

July 5, 1932.

A. O. JOHNSON

1,866,110

METHOD OF FORMING DECORATED METAL OBJECTS

Filed Oct. 14, 1931



*Fig. 2.*



*Inventor:*  
A. O. Johnson,  
by Wm F. Freudenreich, *Atty.*

## UNITED STATES PATENT OFFICE

ALVIN O. JOHNSON, OF CHICAGO, ILLINOIS, ASSIGNOR TO THE MEYERCORD COMPANY,  
A CORPORATION OF ILLINOIS

## METHOD OF FORMING DECORATED METAL OBJECTS

Application filed October 14, 1931. Serial No. 568,869.

The present application is a continuation in part of my prior application Serial No. 553,484, filed July 27, 1931.

The present invention relates to the art of 5 decorating metal to give it any desired surface ornamentation; and it has for its object to produce a simple and novel method of producing the desired surface ornamentation through decorative coatings which shall 10 be tough and elastic and, in effect, form an integral part of the structure as a whole.

There is a large field in which sheet metal objects have been formed or shaped so as no longer to be flat, and must carry surface 15 ornamentation. Viewed in one of its aspects, the present invention may be said to have for its object so to cover surfaces of metal sheets with tough, elastic, decorative coatings that the sheets may be worked or formed in dies 20 into desired shapes without damaging the decorations.

In carrying out my invention, I first apply to the metal surface a ground coat which will ordinarily, but not necessarily in every instance, be pigmented with suitable colors. If 25 the nature of the decoration or ornamentation is such that rare woods, for example, are to be imitated, the pigment in this ground coat will correspond in color to the ground 30 colors of the woods. The ornamental effect or design is then completed by the imposition upon the ground coat of a printed or lithographed transfer or decalcomania. Where 35 woods are to be imitated, the transfers or decalcomanias will represent the grain of the wood. After the decorating has been completed, as will be explained more in detail hereafter, the sheets may be worked or formed in dies.

40 It is a comparatively simple matter to decorate a flat metal surface with a decalcomania or transfer, but great difficulty has always been experienced in producing a product of this kind which will stand up under the operation of shaping the sheet metal in dies or 45 otherwise. The commercial practice in this respect has been to leave the paper backings of the transfers or decalcomanias in place after application has been made to the metal, 50 in order that the paper might protect the

decorations during the forming processes. However, various difficulties are encountered by reason of the presence of the paper during the forming operations. Viewed in one of its aspects, my invention may be said to have for its object to decorate a metal sheet with a paint or color film or films in such a manner that the sheet may be bent or drawn or be otherwise worked after the paper backing of the transfer or decalcomania has been 55 removed and without requiring the presence of the backing to protect the decoration or ornamentation while the sheet is being worked.

The present invention is illustrated more 60 or less diagrammatically in the accompanying drawing, wherein:

Figure 1 is a perspective view of a sheet of metal to which there has been applied a decalcomania, the paper backing still remaining, and portions being broken away to expose all of the various layers; and Fig. 2 is an elevation showing conventionally a set of bending dies about to close on a decorated metal sheet to bend the sheet.

The ground coat must be of such a character that, at the end of the decorating process, it will adhere tenaciously to the metal and be tough and elastic. I have successfully used for this purpose a varnish composed of synthetic gums ground in oils and pigmented with colors where a colored ground coat is desired. However, the ground coat may have as a base other substances, compounds, or mixtures as, for example, synthetic resin or 80 pyroxylin. The color film that is to go on this ground coat may be made in oil colors or mineral pigments produced by printing or lithographing upon transfer paper coated with a water-soluble gum.

When the color film is to be attached, the ground coat is made tacky, or somewhat yielding, plastic or impressionable through the application of a suitable substance, compound or mixture, of a character depending on the 85 type of ground coat. This substance, compound or mixture may be applied directly to the ground coat; it may be applied to the color film in which case it does not come in contact with the ground coat until the color 90 95 100

film is laid on the ground coat; or it may be applied to both the ground coat and the color film. In actual practice good results have been obtained with substances made in accordance with each of the following formulæ:

10 A. 2½ gallons of ethyl lactate; 1¼ gallons of ethylenechlorhydrin; ¼ gallon of ethyl alcohol; and in the neighborhood of 1 gallon of pure clean water. The last three ingredients are preferably mixed together and the ethyl lactate added last.

15 B. 30 parts of methyl alcohol; 30 parts of mono-ethyl ether of ethylene; and 40 parts of water.

20 Since the products of the above formulæ are in liquid form, the simplest way of applying them is simply to dip the transfer into the liquid and then to lay it, color side down, on the ground coat, the paper backing being, of course, uppermost. The transfer or decalcomania is then pressed flat and into intimate contact with the ground coat, preferably by means of roller pressure. The product is 25 then allowed to dry and, after drying, the paper backing is removed in the usual way and any gum left on the color film is washed off so as to leave a clean surface. After this, the sheet is baked for a considerable time. I 30 have obtained good results by baking for a period of from one hour to an hour and a half at a temperature in the neighborhood of 250° F., but the time, as well as the temperature, may be varied.

35 The process of applying the decalcomanias to the metal may be a continuous one, the decalcomanias being employed in long strip or roll form and being drawn through the liquid just before being passed between pressure 40 rolls along with the coated metal.

45 When the sheet is removed from the baking oven, the coatings on the metal form a single tough, elastic layer which adheres to the metal so effectively that the metal may be bent or drawn without cracking the decorative layer or coating and without in any way marring the appearance of the latter. Therefore, the sheet may be placed in forming dies and formed in the usual way, just as though it 50 were a plain sheet of metal.

55 It is not necessary that the product, when it leaves the baking oven, have a polished surface, it being sufficient that the decorative coating be of a character that will permit lacquer or the like to be sprayed over the same before the object is put to its final use.

60 So far as I am aware, I am the first successfully to bend sharply or work up in forming dies comparatively thick metal sheets decorated with printed or lithographed transfers or decalcomanias in oil colors or pigments, without employing some protective layer or covering for the decoration during the shaping or forming operation.

65 As heretofore stated, the substance, com-

70 pound or mixture by which the design is caused to be united to the ground coat is of a character to render the ground coat tacky or somewhat yielding, plastic or impressionable, whereby, under the pressure subsequently applied, the design becomes firmly united to the ground coat. Then, by the baking operation, the ground coat and the design become integrated into a single body; the baking, of course, also altering the character of the composite coating to harden and toughen it without rendering it brittle or altering the design.

75 In Figure 1 of the drawing, 1 represents a sheet of metal and 2 the ground coat thereon. Laid upon the ground coat, face down, is a 80 decalcomania consisting of a paint or ink film 3 printed in the usual way on a water-soluble gum coating on a paper backing 4. Before the decalcomania is applied provision is made for the presence of a medium between the 85 ground coat and the decorative paint or ink film to bring about an effective union between the said film and the ground coat, as heretofore explained. This material is represented in the drawing by the layer 5.

90 While the decorated metal sheet in its final complete state in a flat form may be worked up in various ways, I have, in Fig. 2 of the drawing, illustrated only one type of working,—a simple bending operation. Referring to this figure of the drawing, A and B are upper and lower dies adapted to bend a flat sheet into a trough-like form. Thus, when a decorated sheet C is placed between the dies and they are closed, the side portions 95 of the sheet are bent down at right angles to the plane of the central portion as indicated in dotted lines at c.

100 I desire that it be understood that the present invention is not limited to that which is illustrated in the drawing, as I intend to be limited only to the extent indicated by the definitions of my invention, constituting the appended claims.

105 I claim:

110 1. The method of decorating a metal object, which consists in applying thereto a ground coat, laying on the ground coat a printed or lithographed design secured to a 115 gum coating on a paper backing, with a substance, compound or mixture of a character to render the ground coat tacky or somewhat yielding, plastic or impressionable interposed between the ground coat and the design, pressing the design against the ground coat, 120 removing the backing, and baking the product.

125 2. The method of producing a decorated sheet metal object, which consists in applying thereto a varnish ground coat, laying on the ground coat a printed or lithographed design secured to a gum coating on a paper backing, with a substance, compound or mixture of a character to render the ground coat tacky or somewhat yielding, plastic or im- 130

pressionable interposed between the ground coat and the design, pressing the design against the ground coat, drying, removing the paper backing, baking the decorated sheet, and forming the sheet in dies.

3. The method of decorating a metal object, which consists in applying thereto a ground coat comprising synthetic gums or resins ground in oil, dipping in a liquid composed of ethyl lactate, ethylenechlorhydrin, ethyl alcohol and water, a printed or lithographed design secured to a gum coating on a paper backing, laying the design face down on the ground coat, applying pressure, removing the backing, and baking the decorated object.

4. The method of producing a sheet metal decorated object, which consists in applying to a metal sheet a varnish ground coat comprising synthetic gums or resins ground in oil and pigmented with colors, dipping in a liquid composed of ethyl lactate, ethylenechlorhydrin, ethyl alcohol and water a printed or lithographed design secured to a gum coating on a paper backing, laying the design face down on the ground coat, applying pressure, removing the backing, baking the decorated sheet, and then forming the sheet into the desired shape.

5. The method of decorating a metal object, which consists in applying thereto a ground coat, laying on the ground coat a printed or lithographed design secured to a gum coating on a paper backing, with a substance, compound or mixture of a character to render the ground coat tacky or somewhat yielding, plastic or impressionable interposed between the ground coat and the design, pressing the design against the ground coat, removing the backing, and baking the product for an hour or more at a temperature of about 250° F.

6. The method of producing a decorated sheet metal object, which consists in applying thereto a varnish ground coat pigmented with colors, laying on the ground coat a printed or lithographed design secured to a gum coating on a paper backing, with a substance, compound or mixture of a character to render the ground coat tacky or somewhat yielding, plastic or impressionable interposed between the ground coat and the design, pressing the design against the ground coat, drying, removing the paper backing, baking the decorated sheet for an hour or more at a temperature of about 250° F., and forming the sheet in dies.

7. The method of decorating a metal object, which consists in applying thereto a ground coat pigmented with colors, laying on the ground coat with an interposed layer of a substance, compound or mixture capable of rendering the ground coat tacky a printed or lithographed design secured to a gum coating on a paper backing, pressing the design

against the ground coat, removing the backing, and baking the product.

8. The method of producing a decorated sheet metal object, which consists in applying thereto a ground coat, laying on the ground coat a printed or lithographed design secured to a gum coating on a paper backing, with a substance, compound or mixture capable of causing the design to become united with the ground coat interposed between the ground coat and the design, pressing the design against the ground coat, drying, removing the paper backing, baking the decorated sheet, and forming the sheet in dies.

9. The method of decorating a metal object, which consists in applying thereto a ground coat, dipping a printed or lithographed design secured to a gum coating on a paper backing in a liquid substance, compound or mixture of a character that will cause the design to become united with the ground coat, laying the design face down on the ground coat, applying pressure, removing the backing, and baking the decorated object.

In witness whereof, I sign this specification.

ALVIN O. JOHNSON.

85

100

105

110

115

120

125

130